

Patented Mar. 2, 1926.

1,575,143

# UNITED STATES PATENT OFFICE.

MURRAY C. BEEBE AND ALEXANDER MURRAY, OF CINCINNATI, OHIO, ASSIGNORS TO THE WADSWORTH WATCH CASE COMPANY, OF DAYTON, KENTUCKY, A CORPORATION.

## PHOTOGRAPHIC SENSITIZER.

No Drawing.

Application filed November 18, 1922 Serial No. 601,885.

To all whom it may concern:

Be it known that we, MURRAY C. BEEBE, a citizen of the United States, and ALEXANDER MURRAY, a subject of the King of Great Britain, both residing at Cincinnati, in the county of Hamilton and State of Ohio, have invented certain new and useful Improvements in Photographic Sensitizers, of which the following is a specification.

10 Our invention relates to improvements in photographic sensitizers and it more especially consists of the features pointed out in the annexed claims.

The purpose of our invention is to provide 15 a photographic sensitizer which may be used with various organic bases to produce prints by inducing and accelerating physical changes in the base selectively in accordance with a luminous image; that utilizes chemi-

20 cals heretofore found unavailable for photographic uses; that accomplishes results hitherto unattained; that further provides a means of using a colloidal metallic iodide in combination with a protective colloid for 25 photo-sensitizing a hydrophobic organic colloid; and that provides a stable sensitizer which may be combined with the medium or base and kept in the dark for comparatively long periods without deteriorating.

30 With these and other ends in view, we set forth such steps and relation of steps and the use of various ingredients, as an instance of adaptation of the broad underlying features of our invention without 35 limiting ourselves to the specific exemplifications described herein.

In practically carrying out our invention, we first mix a solution of an organo-metallic compound with a protective colloid and then 40 add a source of halogen which constitutes the photo-sensitizing agent.

The metallic compound reacts with the halogen compound to produce a metallic halide which although insoluble in the dis- 45 persive medium is prevented from separating out by the peptizing action of the protective colloid.

In practice we use an organo-metallic compound, such as metal alkyls, for instance, of lead, silver, mercury, nickel, etc., a typical example of this class is lead triethyl iodide or the metal ethereal salts of which lead tungate is an example, or their equivalents, with a protective colloid, exemplified by all colloidal organic materials,

such as thickened oils, cellulose acetate, resins, bitumens, etc., combined with a halogen source which may consist of free halogens, such as iodine, bromine, or mixed halogens, or soluble halides such as the organo-iodides; 60 the following may be instanced as examples of the latter, idoform, ethylene iodide, etc., as sources of halogen the organo-bromides are also cooperatively available.

As an example of usage, without limiting 65 ourselves to a specific procedure we have found the following sensitizer to give practical results:

Organometallic compound—4.2 gms. lead triethyl iodide in 30 cc. benzene. 70

Protective colloid—3 gms. asphaltum in 15 cc. solvent naphtha.

Halogen source—3 gms. idoform in 20 cc. ethyl methyl ketone.

To produce a photo-sensitive coating 25 75 cc. of a suitable varnish is added to the above with which a metallic plate is coated and the solvent is allowed to evaporate. When an oleaginous varnish is used the plates are available as wet plates for direct 80 optical projection and if a gum-varnish is used the plates when dry may be used for contact printing. After the prints are made they are developed in any desired solvent which will remove the unacted parts of the 85 coating proportional to the variable action of light.

The term protective colloid as used herein includes all substances having peptizing characteristics or any substance which has 90 the power of keeping the metallic halide in such a high state of dispersion that it resembles a solution and which is permanently stable, showing no precipitation. Also the term hydrophobic organic colloid as used herein is a colloidal substance which is dispersed in a solvent other than water. It is however possible to add minor quantities of water to some of the sols. In using the hydrophobic designation we do not limit ourselves to an absolute absence of water. Our use of "organosol" is synonymous with colloidal sol in which the dispersing medium is an organic substance. 100

Prior practice and procedure with halogen sensitizers has invariably been accompanied by their rapid deterioration, making it impossible to use them, in a prepared state longer than one or two days. In fact the highly sensitive mediums will only remain 110

stable for a few hours. Our present sensitizer shows a stability far in excess of any used heretofore, continuing usable indefinitely.

5 The speed of our sensitizer is quite rapid, for same size copying, when incorporated with a suitable medium in 10 seconds and when used in connection with optical projection at an enlargement of 190:1 areas the 10 time is increased only to 10 minutes producing easily developed and clean images.

If saponaceous solvents are used as developers of prints on electropositive metals an adsorbed film of fatty acids remains in 15 the high lights as a "seum" preventing clear high lights in the prints. With our present sensitizer and the use of a petroleum or turpentine, single solvent, all indications of seum are removed.

20 What we claim is:

1. A photographic sensitizer adapted for sensitizing a photographic medium, said sensitizer comprising a hydrophobic protective colloid, and a metallic halide and a halogen-liberating compound dispersed therein.

25 2. A photographic sensitizer adapted for

sensitizing a photographic medium, said sensitizer comprising a hydrophobic protective colloid, and a metallic halide dispersed therein.

30

3. A photographic sensitizer adapted for sensitizing a photographic medium, said sensitizer comprising a hydrophobic protective colloid, and a metallic halide and another halogen-liberating compound dispersed in said protective colloid.

35 4. A photographic sensitizer adapted for sensitizing a photographic medium, said sensitizer comprising a hydrophobic protective colloid, and a metallic halide and a halogen-liberating organic compound dispersed in said protective colloid.

40 5. A photographic sensitizer adapted for sensitizing a photographic medium, said sensitizer comprising a hydrophobic protective colloid, and a metallic halide and iodoform dispersed in said protective colloid.

45 In testimony whereof we affix our signatures.

MURRAY C. BEEBE.  
ALEXANDER MURRAY.